

Aug. 8, 1933.

K. L. MEISSNER

1,921,089

ALUMINUM ALLOY

Filed March 30, 1931



INVENTOR

Karl L. Meissner,

Watson, Cut, Moore & Grindell  
Attns

## UNITED STATES PATENT OFFICE

1,921,089

## ALUMINUM ALLOY

Karl Leo Meissner, Duren, Germany, assignor  
to Durener Metallwerke Aktiengesellschaft,  
Duren, Germany, a German joint stock Com-  
pany

Application March 30, 1931, Serial No. 526,525,  
and in Germany April 1, 1930

3 Claims. (Cl. 148—21.1)

It is known that further increases in the yield point beyond the values obtained by the natural aging of self tempering aluminum alloys may be obtained in the following way:

- 5 1. By the generally known process of cold working which is applicable not only to aluminum alloys that may be tempered but quite generally to all practically deformable metals and alloys.
- 10 2. By the use of the so-called artificial aging, i. e., a heat hardening process carried out at moderately high temperatures. Such a process is disclosed, for example, in the French Specification No. 555,836, Leichtmetall Studien und Ver-  
15 wertungs Gesellschaft m. b. H. of April 3, 1923, or in the United States Patent No. 1,695,044 to Hallmann, granted December 11, 1928, there being, however, as compared with the process according to the present invention, a difference inasmuch as in the first place, cold working is employed not before natural aging is complete but at an earlier point, and also in that the temperatures employed for annealing lie above the critical aging temperature, so that they do not attain 20 the desired object in the process according to the present invention.

Both the known processes described in the foregoing have the disadvantage that the increase in the yield point is accompanied by a diminution in the elongation and a decline in other very valuable technical and chemical properties; above all, ductility, concavity and reduction in cross-section deteriorate, and the resistance to corrosion likewise falls. It is a peculiarity of the effect of artificial aging that the falling off in the aforementioned properties begins just at the moment when the yield point commences to rise. For these reasons, a technical gain cannot be noted either with the one or the other of the known processes, because the one-sided improvement of the alloy can only be secured at the expense of several other likewise valuable mechanical and chemical properties.

A process is also known which is chiefly employed in the manufacture of wire of high electrical conductivity from aluminum alloys and wherein the rolled or extruded wire is heated to high temperatures, is quenched and is thereupon subjected, without long natural aging, to a very extensive cold working by drawing, the wire being thereupon annealed at a temperature below 250° C. until the desired conductivity is attained. This process differs from that according to the present invention by the very important feature 55 that no storing is provided after quenching and

moreover also in that the cold working by drawing is very much greater than in the present process, being namely about 95%.

A process relating to the same wire alloy for overhead conductors is employed to increase the 60 yield point and elastic limit, whereby the finished drawn wire is stretched, after annealing, by 0.5 to 2% and is then re-annealed at 50—160° C. This process likewise differs in the following way from that according to the present invention. 65

Due to the pretreatment described in the foregoing which departs entirely from that of the present invention, the wire is in quite a different condition from the outset, and consequently also, in the stretching of the wire, the subsequent annealing treatment causes a further rise in the yield point and elastic limit, whereas in the process according to the present invention, it is just the reverse, the annealing treatment being carried out within such a temperature range that 70 these properties decline again to a minimum value. The individual steps of the processes differ entirely, therefore, both as regards their nature and their effect. 75

In a publication by L. Guillet, "Revue de 80 Métallurgie" vol. 23 (1926) pp. 48—52, there is described, inter alia, a test on duralumin, whereby the material was heated, quenched and then subjected to cold working. This test, however, lacked the most important feature of the present invention, namely, the subsequent annealing at such temperatures and for such lengths of time that the elongation lowered by the cold working is raised again to the value of the naturally aged alloy while preserving, at the same time, an increased yield point. 85

In the United States Patent No. 1,472,739, granted October 30, 1923 to R. S. Archer and Z. Jeffries, it is stated that an alloy of 0.5% magnesium and 0.75% silicon, after quenching from 95 550° C. was stretched by 15% in a machine for testing tensile strength and was thereupon aged artificially for 60 hours at 145° C. After this treatment the alloy exhibited certain properties of tensile strength, elongation and Brinell hardness. It is also stated in the specification that the alloy exhibited similar final properties when the quenched alloy was first aged at room temperature and then stretched 15% and aged artificially for 60 hours at 145° C. From this observation alone, namely, that as regards the attainment of the final properties, it was immaterial whether aging at room temperature was included or not before stretching, it may be gathered that the method disclosed in the said specification 100 105 110

differs from the present invention according to which an important part is played by the sequence of the individual steps, and more particularly in the complete natural aging before cold working.

That this is the case is not anticipated, however, by the aforementioned specification, and is also not recognized in the invention contained therein, because the after-treatment is carried out in such a way that essentially different properties are thereby obtained, which completely mask the effect of a previous aging at room temperature. In the comparatively long space of time of 60 hours, the temperature of 145° C. is not considerably higher than the range at which the present invention results in its success. At this high temperature, combined with such a long space of time, a pronounced effect of artificial aging is concerned, and this term is also expressly employed in the specification as follows also from the elongation of 12.5%, which is remarkably low for such a slightly alloyed composition. In the naturally aged condition, however, the alloy has an elongation of 37.5%. According to the present invention, the procedure is such that the elongation is raised again to the normal value, whereas it follows from the statement made in the United States specification that the elongation in the treatment described falls to  $\frac{1}{3}$  of the normal value.

In contradistinction to the known processes described in the foregoing, it is the object of the present invention to attain an increase in the yield point with simultaneous moderate increase in the tensile strength, without at the same time having any detrimental effect on the elongation and on the other properties mentioned in the foregoing, namely, deformability and resistance to corrosion. The two examples hereunder will serve to explain the essential features of the invention.

An alloy with 4.2% copper, 0.5% magnesium, 0.25% manganese and about 0.25-0.3% each of iron and silicon as impurities gave in the improved or heat treated condition a yield point of about 25 kg/mm<sup>2</sup>, a tensile strength of about 40-42 kg/mm<sup>2</sup> and an elongation of about 20-22%. When this alloy, after natural aging was further annealed at high temperatures, i. e. was subjected to the process of artificial aging, a drop in the yield point and also in the tensile strength, attaining a minimum value with an aging period of 20 to 40 hours at about 100° C., was observed in the temperature ranges at which no diminution in the elongation and ductility could yet be detected. The yield point fell to about 21-22, and the tensile strength to about 37-38 kg./mm<sup>2</sup>. The behavior of the yield point in this experiment may be gathered from the dotted line curves in Figure 1.

The case was somewhat the same when the alloy was subjected to the same treatment immediately after quenching from the high temperature treatment. Here again a drop in the yield point and tensile strength was observed, the yield point at 100-125° C. falling to about 22-24, and the tensile strength to about 38-39 kg/mm<sup>2</sup>. The behavior of the yield point in this series of experiments will be seen from the chain line curve in Figure 1. Both sets of curves substantially agree with one another.

Thus, the annealing treatment, in the temperature regions where the elongation and deformability still remain unchanged, resulted in no technical advantage, there being a drop in the yield

point and tensile strength in these temperature regions.

However, when still higher temperatures were employed at which the yield point and also to some extent the tensile strength increase, it is likewise not possible to attain a technical advantage, as already explained in the foregoing, because the elongation and deformability are likewise unfavorably affected by the same treatment.

The same alloy, after completion of natural aging, was now cold worked, the yield point being reduced to about 37-38 and the tensile strength to about 46-47 kg/mm<sup>2</sup>, while the elongation fell in this treatment to about 15-17%. On employing artificial aging on an alloy pretreated in this manner, it was unexpectedly found that, on employing the same aging period of 20 to 40 hours, the yield point and tensile strength fell, reaching a minimum at about the same temperatures of 100-125° C., but that the drop only went so far as such values as lie about 40% and more above those obtained at the same temperatures in the two instances mentioned in the foregoing. In addition, these minimum values lay about 20-30% higher than the values exhibited by the yield point of the merely improved alloy. In the temperature ranges of 100-125° C., yield point values of 30-33 kg/mm<sup>2</sup> were obtained (see full line curve in Figure 1). At the same time, the tensile strength was 42-44 kg/mm<sup>2</sup>, i. e. it also lay about 5% higher than in the merely improved state and about 10-15% higher than the corresponding minimum values which were obtained at the same temperatures with inclusion of the cold working. At the same time, the elongation, which had been reduced by cold working, rose again to about 21% (see Figure 2).

A magnesium free aluminum alloy with about 5.8% copper, 0.7% manganese and again the usual impurities in the form of iron and silicon had, in the improved condition, a yield point of 27.4 kg/mm<sup>2</sup>, a tensile strength of 40.8 kg/mm<sup>2</sup> and an elongation of 16.2%. Since this alloy, as compared with magnesium-containing alloy mentioned in the first example, did not possess the feature of self-improving on standing at the room temperature, the alloy, after being quenched from high temperature treatment, was further tempered for 24 hours at 145° C. In this condition it was approximately comparable with the naturally aged condition of a magnesium-containing alloy. The alloy so treated having the above-mentioned properties was now cold worked and then annealed 20 hours at 110° C. The yield point was then 33.4 kg/mm<sup>2</sup>, the tensile strength 43.1 kg/mm<sup>2</sup> while the elongation had again gone up to 16.5%.

It may be stated with respect to the magnesium content that in these age-hardenable alloys amounts of magnesium in excess of 2% are generally recognized as affording no advantage, and thus when speaking of an age-hardenable alloy it is understood that the magnesium content does not exceed this limit. Thus in the Zeitschrift fur Flugtechnik und Motorluftschiffahrt, vol. 17, 1926, page 114, it is explained that the magnesium content of duralumin, a recognized age-hardenable aluminum alloy, should not in practice exceed 2%, since otherwise the age-hardening effect becomes smaller.

It is already known that the effect of cold working may be removed again by subsequent annealing and that the alloy may be made soft again, the properties of strength falling and the

elongation and deformability rising. For the alloys in question, this region lies generally at temperatures of about 350-400° C. The process according to the present invention differs, however, 5 from this generally known annealing process in that, in the present process, it is not a question of a purely annealing effect but of a peculiar combination of annealing treatment and of an effect of artificial aging, which certainly only occurs 10 in a very narrow temperature range, which in the examples described in the foregoing lay at about 100-125° C.

The effect of this combination in the narrow temperature range in question is that the elongation, as in annealing, again rises to its normal 15 original values, while obviously in the case of the yield point and also the tensile strength, the effect of the annealing is partly covered by the artificial aging. Since at the same time and at 20 the same temperatures, the deformability and the elongation both attain their maximum values, and a renewed falling off in these properties only occurs when the above-mentioned temperature 25 limit is exceeded, the application of the process depicted, in the individual steps as described in the examples, provides on the whole a technical advantage, because a higher yield point with 30 moderately increased tensile strength is now imparted to the material while preserving, however, the high values for the elongation and deformability, such as could not be imparted to it

in this combination and at the same time in the processes known heretofore.

I claim:—

1. In the tempering of age-hardenable aluminum alloys containing magnesium in an amount not exceeding 2%, the process of increasing the elongation while preserving at the same time a high yield point consisting in annealing for twenty to forty hours at a temperature of about 100°-125° C. after the alloy has been heated to 80 the high temperature, quenched, completely aged at room temperature and cold worked.

2. In the tempering of age-hardenable aluminum alloys containing about 0.5% magnesium and about 4.2% copper, the process of increasing the elongation while preserving at the same time a high yield point consisting in annealing for 20 to 40 hours at a temperature of about 100°-125° C. after the alloy has been heated to the high temperature, quenched, completely aged at room 85 temperature and cold worked.

3. In the tempering of age-hardenable aluminum alloys containing about 0.5% magnesium, about .25% of manganese, and about 4.2% copper, the process of increasing the elongation 100 while preserving at the same time a high yield point consisting in annealing for 20 to 40 hours at a temperature of about 100°-125° C. after the alloy has been heated to the high temperature, quenched, completely aged at room temperature 105 and cold worked.

KARL LEO MEISSNER.

35

110

40

115

45

120

50

125

55

130

60

135

65

140

70

145

75

150